

## UNITED STATES PATENT OFFICE

2,684,334

LUBRICATING OIL CONTAINING A REACTION PRODUCT OF  $P_2S_5$ -TERPENE AND 2,4,6-TRIALKYLPHENOL

Julian G. Ryan and George L. Hayes, Wood River, Ill., assignors to Shell Development Company, Emeryville, Calif., a corporation of Delaware

No Drawing. Application May 25, 1951,  
Serial No. 228,356

15 Claims. (Cl. 252—46.6)

1

This invention relates to improved lubricating compositions particularly for use in aviation and similar types of engines.

The problem of engine fouling, corrosion and the like, is particularly acute in aviation engines, in which the high temperatures developed in the cylinders tend to act upon lubricating oils to cause the deposition of resinous and varnish-like products on the pistons and elsewhere and to produce lacquer-like coatings and carbonaceous materials, which in time tend to cause ring and valve sticking and interfere with engine operation. High piston temperatures in aviation engines promote the formation of deposits which, in turn, aggravate the situation by reducing the heat transfer. Furthermore, fuel residues from incomplete combustion of fuel contribute to the deposition of lacquer-like and carbonaceous materials in the engine.

Accordingly, it is an object of this invention to provide lubricating oil compositions which have improved properties in one or more of the following qualities: high temperature detergency, decreased piston ring sticking, wear reduction, corrosion resistance, stability in presence of copper or crankcase catalyst, oxidation stability, and the like. Another purpose is to produce a superior heavy duty lubricant particularly suitable for use in aircraft and other internal combustion engines operating at relatively high cylinder temperatures. Other objects will be apparent from the following description.

It has now been found that such lubricating problems can be substantially overcome by the incorporation in a lubricating oil base, of minor amounts, but in critical and mutually coating proportions, of two particular types of non-ash-forming additives, the combination of which with the base lubricant exerts a synergistic effect, resulting in a composition of outstanding stability and lubricity.

One of the additives of the combination is a 2,4,6 trisubstituted polar containing aromatic compound represented by the general formula:



wherein Ar is a mono- or dinuclear aromatic radical, R is the same or different organic radicals attached to nuclear carbon atoms, at least one of said R's being an alkyl radical ortho in position to a YH radical and linked to the ring carbon atom by a tertiary carbon in the alkyl group and the remaining R's being the same as the R which is ortho to YH radical or they can be the same or different essentially alkyl, aralkyl,

2

cycloalkyl hydrocarbon radicals containing if desired minor proportions of polar substituents, e. g.,  $NO_2$ ,  $NH_2$ ,  $OH$ ,  $SO_3H$ ,  $COOH$ ,  $CN$ , etc., Y is a chalcogen element having an atomic number of 8 to 16, namely, oxygen and sulfur (yielding the phenols and thiophenols), the radicals (YH) being attached directly to the aromatic ring, x is an integer of 1 to 2 and y is an integer of at least 3. If x is greater than one, then the radicals YH can be the same or different.

A preferred embodiment of additives within the class as broadly defined by formula I are 2,4,6, trisubstituted phenols represented by the formula:

15



(II)

20

wherein  $R_1$  is a tertiary alkyl radical such as tertiary butyl, tertiary amyl, 1,1,3,3-tetramethylbutyl, and the like, preferably containing up to about 12 carbon atoms, one of  $R_2$  and  $R_3$  is a

25

hydrocarbon radical, preferably an alkyl radical, either a primary, secondary or tertiary alkyl radical, while the other one is the same or different hydrocarbon radical as defined or an aromatic-substituted alkyl radical, more particularly an ortho- or para-hydroxy-alkyl phenyl-substituted alkyl (ortho-hydroxy-alkyl benzyl-) radical, being the ortho-isomer when it is  $R_2$  and the para-isomer when it is  $R_3$ .

30

When  $R_2$  or  $R_3$  is an ortho- or para-hydroxy-alkyl phenyl-substituted alkyl radical, respectively, the alkyl substituents thereof are chosen to be identical with  $R_1$  and the other one of  $R_2$  and  $R_3$ ; thus, the compounds are alkylene bis(alkylphenols).

35

Specific examples of compounds represented by the above formula and which are particularly useful in the practice of this invention are:

2,6-ditertiary butyl-4-methylphenol  
2,4-ditertiary butyl-6-methylphenol  
2,4-dimethyl-6-tertiary-butylphenol

45 2,6-di-sec-butyl-6-tertiary-butylphenol  
2,4-di-n-butyl-6-tertiary-octylphenol

2,6-ditertiary-butyl-4-benzylphenol  
2,6-ditertiary-amyl-4-methylphenol

2,4-ditertiary-amyl-6-methylphenol

50 2,4,6-tritertiary-butylphenol  
2,6-ditertiary-butyl-4-methylthiophenol

2,4-ditertiary-butyl-6-methylthiophenol  
2,4-dimethyl-6-tertiary-butylthiophenol

2,4-dimethyl-6-tertiary-octylthiophenol

55 2,6-ditertiary-amyl-4-methylthiophenol

## 3

2,4,6-tri-tertiary-amylthiophenol  
 2,2' - methylene bis(4 - methyl - 6 - tertiary-butylphenol)  
 2,2' - methylene bis(4,6-ditertiary-butylphenol)  
 2,2' - methylene bis(4,6-ditertiary-octylphenol)  
 2,2' - methylene bis(4 - methyl - 6 - tertiary-amylphenol)  
 2,2' - methylene bis(4 - methyl - 6 - tertiary-octylphenol)  
 2,2' - methylene bis(4 - methyl - 6 - tertiary-butylthiophenol)  
 2,2' - methylene bis(4 - octyl-6-tertiary-butylthiophenol)  
 2,2' - methylene bis(4,6 - ditertiary - butylthiophenol)  
 2,2' - methylene bis(4,6 - ditertiary - amylthiophenol)  
 2,2' - methylene bis(4 - methyl - 6 - tertiary-amylthiophenol)  
 2,2' - methylene bis(4 - methyl - 6 - tertiary-octylthiophenol)  
 (2 - hydroxy - 3 - tertiary - butyl - 5 - methylphenyl) - furylmethane  
 (2 - hydroxy - 5 - tertiary - butylphenyl) - furylmethane  
 1,1 - bis(2 - hydroxy - 3 - tertiary - butyl - 5 - methylphenyl) isobutane  
 Bis(2 - hydroxy - 3 - tertiary - butyl - 5 - methylphenyl) phenylmethane  
 2,2 - bis(2 - hydroxy - 3 - tertiary - butyl - 5 - methylphenyl) propane  
 2,2 - bis(2 - hydroxy - 3 - tertiary - butyl - 5 - methylphenyl) butane

The trisubstituted phenolic compounds and mixtures thereof can be used in amounts varying from 0.01 to about 10% and preferably from 0.1 to 5% by weight, with from 0.5% to 3% by weight being a still more preferred range.

The second additive used in lubricating compositions of this invention is a phosphorized terpene compound obtained as a reaction product by reacting a terpene compound with a phosphorizing agent. Terpenes suitable for producing reaction products of this invention include alpha- and beta-pinene, dipentene, terpinolene, menthene, alpha-terpineol, camphene, limonene, turpentine, pine oil, camphor oil, terpenes obtained as a by-product in manufacture of synthetic camphor, carene, fenchene, terpinene, di-terpenes, camphoric acid, abietic acid, etc. The phosphorizing agents which can be used to form reaction products of this invention are:  $P_2S_5$ ,  $P_4S_3$ ,  $P_2Se_3$ ,  $P$ ,  $P_2O_5$ ,  $POCl_3$ ,  $PCl_3$ ,  $PCl_5$ ,  $PSCl_3$ , etc. Also the terpene compounds can be first reacted with a sulfurizing agent, e. g.  $SCl_2$ ,  $S_2Cl_2$ , sodium polysulfide,  $SeCl_2$ ,  $SeCl_4$  and the like and thereafter retreated with a phosphorizing agent, e. g.  $P_2O_5$ ,  $P_2S_5$ , phosphoric acid, etc., so that the final reaction product contains both sulfur and phosphorus. If desired, the reaction can be carried out in the reverse order, namely, the terpene compound can be first treated with a phosphorizing agent, e. g.,  $P_2O_5$  and thereafter treated with sulfur, metal polysulfides, sulfur chloride and the like. The reaction can be carried out in an inert diluent such as light hydrocarbons, or in a base oil to which the reaction product is intended to be added.

When the reaction products of this invention are produced in a two-step process, namely, by first sulfurizing and then phosphorizing, the sulfurization temperature can vary from 200 to 400° F. and the phosphorization step can be carried out at the reflux temperature of the reactants.

## 4

With phosphorus sulfides the reaction can be made to proceed at room temperature or higher temperatures depending upon the terpene compound being treated.

5 The mole ratio of the terpene compounds to the phosphorus and sulfur or phosphorizing reagent may vary over wide limits, such as from 10:1, preferably 4:1, to 3:1 moles of the above-mentioned reagents, respectively.

10 The preparation of the reaction products can be effected by heating a terpene compound to an elevated temperature of around 200° F. or higher and slowly adding the phosphorizing agent. After the addition is completed, the temperature of the reaction is increased to 250-400° F. and preferably is maintained between 300 and 350° F. until all of the phosphorizing agent such as  $P_2S_5$  has reacted and evolution of hydrogen sulfide ceases. If desired, the reaction product can be purified or refined by solvent treatment or neutralized by treatment with a nitrogen base.

15 It is preferred to utilize the phosphorized and sulfurized terpene compound, as such, in the present compositions. However, they can be neutralized and/or reacted with organic nitrogen base compounds such as amines and quaternary ammonium compounds, as illustrated by tri-  
 20 amylamine, triethanolamine, laurylamine, octadecylamine, morpholine, dibutylamine, dicyclohexylamine, trimethylhexylammonium hydroxide, dibenzylamine, methylaniline, trimethylbenzylammonium hydroxide, piperidine, and the like.

25 35 Specific examples of reaction products under discussion and their detailed method of preparation are as follows:

30 About 4 moles of gum spirits of terpentine was heated under agitation to around 250° F., and about 1 mole of  $P_2S_5$  was added portionwise maintaining the temperature of the mixture around 250° F. until all of the  $P_2S_5$  had been added. The temperature was then increased to 275-300° F. and the mixture reacted until evolution of  $H_2S$  ceased. On analysis the product contained 12.8% S and 4.81% P.

35 Another product was prepared by heating 4 moles of alpha-pinene with 1 mole of  $P_2S_5$  at around 240° F. until all of the  $P_2S_5$  had been added and thereafter increasing the reaction temperature to around 300° F. and maintaining the mixture at said temperature until the reaction was completed. On analysis the product contained 12.7% S and 4.62% P.

40 55 The above reaction products can be modified by treating them with amines of which the long chain alkyl amines, e. g., octadecylamine and laurylamine, are preferred.

50 The phosphorized-terpene compound reaction product can be used in amounts varying from 0.01 to 10% and preferably between 0.1 and 5% by weight, with from 0.5% to 1.0% representing a still more preferred range.

55 60 The base for additives of this invention can be any natural or synthetic material having lubricating properties. Thus, the base may be a hydrocarbon oil of wide viscosity range, e. g., 100 SUS at 100° F. to 150 SUS at 210° F. The hydrocarbon oils may be blended with fixed oils such as castor oil, lard oil and the like, and/or with synthetic lubricants such as polymerized olefins, copolymers of alkylene glycols and oxides; organic esters of polybasic organic and inorganic acids, e. g., di-2-ethylhexyl sebacate, dioctyl 70 phthalate, trioctyl phosphate; polymeric tetra-

hydrofuran; polyalkyl silicone polymers, e. g., dimethyl silicone polymer and the like. If desired, the synthetic lubricants may be used as the sole base lubricant or admixed with fixed oils and their derivatives.

Lubricating compositions of this invention are particularly useful in aviation engines operating on leaded fuels containing a halohydrocarbon scavenger such as ethylene dibromide, with or without the presence of an organic phosphate, e. g., tricresylphosphate.

Illustrative examples of final compositions of this invention in a refined mineral oil base having the properties as indicated below are set forth as Compositions A-J.

#### PROPERTIES OF THE BASE MINERAL OIL

|                                          |       |
|------------------------------------------|-------|
| Gr., ° API                               | 28.5  |
| Color, NPA                               | 4 1/2 |
| Pour point, ° F                          | 10    |
| Flash, ° F                               | 470   |
| Fire, ° F                                | 560   |
| Visc. at 100° F., SSU                    | 1239  |
| Visc. at 210° F., SSU                    | 99.5  |
| Viscosity index                          | 96    |
| Carbon residue, per cent wt. (Conradson) | 0.32  |
| Ash, per cent wt                         | None  |
| Sulfur, per cent wt                      | 0.13  |
| Specific dispersion                      | 109   |

#### Composition A

|                                                            |         |
|------------------------------------------------------------|---------|
| P <sub>2</sub> S <sub>5</sub> -turpentine reaction product | 0.8     |
| 2,6-ditert-butyl-4-methylphenol                            | 1       |
| Mineral lubricating oil                                    | Balance |

The properties of this composition are:

|                                          |       |
|------------------------------------------|-------|
| Gr., ° API                               | 28.3  |
| Color, NPA                               | 5     |
| Pour point, ° F                          | 10    |
| Flash, ° F                               | 470   |
| Fire, ° F                                | 560   |
| Vis. at 100° F., SSU                     | 1150  |
| Vis. at 210° F., SSU                     | 95    |
| Viscosity index                          | 95    |
| Carbon residue, per cent wt. (Conradson) | 0.32  |
| Ash                                      | None  |
| Sulfur                                   | 0.16  |
| Specific dispersion                      | 110.6 |

#### Composition B

|                                                            |         |
|------------------------------------------------------------|---------|
| P <sub>2</sub> S <sub>5</sub> -turpentine reaction product | 0.5     |
| 2,6-ditert-butyl-4-methylphenol                            | 1       |
| Mineral lubricating oil                                    | Balance |

#### Composition C

|                                                            |         |
|------------------------------------------------------------|---------|
| P <sub>2</sub> S <sub>5</sub> -turpentine reaction product | 0.25    |
| 2,6-ditert-butyl-4-methylphenol                            | 1       |
| Mineral lubricating oil                                    | Balance |

#### Composition D

|                                                            |         |
|------------------------------------------------------------|---------|
| P <sub>2</sub> S <sub>5</sub> -turpentine reaction product | 0.8     |
| 2,6-ditert-butyl-4-methylphenol                            | 3       |
| Mineral lubricating oil                                    | Balance |

#### Composition E

|                                                        |         |
|--------------------------------------------------------|---------|
| P <sub>2</sub> S <sub>5</sub> -pinene reaction product | 0.8     |
| 2,6-ditert-butyl-4-methylphenol                        | 1       |
| Mineral lubricating oil                                | Balance |

#### Composition F

|                                                        |         |
|--------------------------------------------------------|---------|
| P <sub>2</sub> S <sub>5</sub> -pinene reaction product | 0.5     |
| 2,6-ditert-butyl-4-methylphenol                        | 1       |
| Mineral lubricating oil                                | Balance |

#### Composition G

|                                                        |         |
|--------------------------------------------------------|---------|
| P <sub>2</sub> S <sub>5</sub> -pinene reaction product | 0.25    |
| 2,6-ditert-butyl-4-methylphenol                        | 1       |
| Mineral lubricating oil                                | Balance |

#### Composition H

|                                                        |         |
|--------------------------------------------------------|---------|
| P <sub>2</sub> S <sub>5</sub> -pinene reaction product | 0.8     |
| 2,6-ditert-butyl-4-methylphenol                        | 3       |
| Mineral lubricating oil                                | Balance |

#### Composition I

|                                                            |         |
|------------------------------------------------------------|---------|
| P <sub>2</sub> S <sub>5</sub> -turpentine reaction product | 0.8     |
| 2,2'-methylene bis(4-methyl-6-tert-butylphenol)            | 1       |
| Mineral lubricating oil                                    | Balance |

#### Composition J

|                                                        |         |
|--------------------------------------------------------|---------|
| P <sub>2</sub> S <sub>5</sub> -pinene reaction product | 0.8     |
| 2,2'-methylene bis(4-methyl-6-tert-butylphenol)        | 1       |
| Mineral lubricating oil                                | Balance |

To illustrate the pronounced improvement obtained using lubricating compositions of this invention in aircraft engines the following tests were made and the data are presented in the table.

I. Compositions of this invention were tested in a Pratt and Whitney R-4360 single-cylinder engine in accordance with the procedure outlined by the Pratt and Whitney Aircraft Corporation for evaluating coking tendency of piston engine lubricating oils by noting the resistance of the oil to high temperature oxidation by temperature stressing the test oil in the exhaust rocker box of an R-4360 cylinder.

II. Compositions of this invention were also tested in a COT engine, developing 8 horsepower at 2400 R. P. M. for 80 hours at the end of which time the condition of the engine was examined and rated.

III. Compositions of this invention were also subjected to the Dornte oxidation test as described in the Industrial and Engineering Chemistry 28, page 26 (1936).

#### TABLE.—TEST RESULTS

##### Dornte oxidation test

[1800 cc., time-minutes, Cu and Fe catalyst.]

| Composition                                                                | Cu Cat. | Fe Cat. |
|----------------------------------------------------------------------------|---------|---------|
| Mineral oil                                                                | 140     | 175     |
| Mineral oil + 1% 2,6-ditert-butyl-4-methylphenol                           | 400     | 340     |
| Mineral oil + .25% P <sub>2</sub> S <sub>5</sub> -terpene reaction product | 480     | 1,480   |
| Composition A                                                              | 680     | 2,480   |
| Composition E                                                              | 680     | 2,480   |

##### Cooperative oil test, CRC project number CLEO-40-46

[Engine (80 hours general performance test).]

| Composition                                                                | Total Engine Rating* | Bearing wt. loss (Mg.) |
|----------------------------------------------------------------------------|----------------------|------------------------|
| Mineral oil                                                                | **12                 | 1,758                  |
| Mineral oil + 1% 2,6-ditert-butyl-4-methylphenol                           | 60                   | 1,555                  |
| Mineral oil + .25% P <sub>2</sub> S <sub>5</sub> -terpene reaction product |                      | 1,502                  |
| Composition B                                                              | 87                   | 38                     |
| Composition F                                                              | 89                   | 24                     |
| Composition H                                                              | 76                   | 33                     |

\*100=perfect; 50=fair; 0=very poor.

\*\*Operation stopped before the 80-hour test because of excess engine fouling.

## Pratt and Whitney R-4360 single-cylinder engine

| Composition      | Results * |
|------------------|-----------|
| Mineral          | 4         |
| Composition Y*   | 6         |
| Composition XX** | 6         |
| Composition C    | 9         |

\*Composition Y = Commercial compounded aviation oil containing Zn salt of alkyl salicylic acid.

\*\*Composition XX = Mineral oil + 1% 2,6-ditertiary-butyl-4-methylphenol.

\* 10 = perfect; 0 = very poor.

Thus, the present invention provides outstanding non-ash-forming lubricating oils for use in aviation engines, which lubricating oils consist essentially of a lubricating oil containing a minor amount each of certain alkylphenols and of a phosphorized-, sulfurized-terpene, to the essential exclusion of other materials. Although the preferred compositions consist essentially of the three components specified, the addition of minor amounts of other additives is advantageous in some applications, additives such as blooming agents, pour point depressants or viscosity improvers, extreme pressure agents, anti-foaming agents and the like. Among the specific additives which can be used are oil-soluble non-ash-forming salts of various nitrogen bases with detergent-forming acids. Organic bases include various nitrogen bases as primary, secondary, tertiary amines and quaternary ammonium bases.

Examples of detergent-forming acids are the various fatty acids of say 10 to 30 carbon atoms, wool fat acids, paraffin wax acids (produced by oxidation of paraffin wax), chlorinated fatty acids, rosin acids, aromatic carboxylic acids including aromatic fatty acids, aromatic hydroxy fatty acids, paraffin wax benzoic acids, various alkyl salicylic acids, phthalic acid mono-esters, aromatic keto acids, aromatic ether acids, and the like.

Extreme pressure agents which may be used comprise: neutral aromatic sulfur compounds of relatively high boiling temperatures such as diaryl sulfides, diaryl disulfides, alkyl aryl disulfides, e. g., diphenyl sulfide, diphenol sulfide, di Cresol sulfide, dixylenol sulfide, methyl butyl diphenol sulfide, dibenzyl sulfide, corresponding di- and tri-sulfides, and the like; sulfurized fatty oils or esters of fatty acids and monohydric alcohols, e. g., sperm oil, jojoba oil, etc.; in which the sulfur is strongly bonded, sulfurized long-chain olefins such as may be obtained by dehydrogenation or cracking of wax; sulfurized-phosphorized fatty oils or acids, phosphorus acid esters having sulfurized organic radicals, such as esters of phosphorus or phosphoric acids with sulfurized hydroxy fatty acids; chlorinated hydrocarbons, such as chlorinated paraffin, aromatic hydrocarbons and chlorinated esters of fatty acids containing the chlorine in other than the alpha position.

Additional ingredients may comprise oil-soluble urea or thiourea derivatives, e. g., urethanes, allophanates, carbazides, carbazones, etc., polyisobutylene polymers, unsaturated polymerized esters of fatty acids and monohydric alcohols and other high molecular weight oil-soluble compounds.

Depending upon the additive used and conditions under which it is used, the amount of additive used may vary from 0.01 to 2% or higher. However, substantial improvement is obtained by using amounts ranging from 0.1 to 0.5% in com-

bination with the two primary additives of this invention.

Compositions of this invention may also be used with motor oils, turbine oils, steam cylinder oils, marine engine oils, refrigeration oils, and used for various lubricating purposes other than engine lubrication, such as slushing and flushing oils, rust inhibiting oils, quenching and drawing oils, greases, wax compositions, and the like.

10 We claim as our invention:

1. A non-ash aviation engine lubricating oil composition having the following formulation:

15 2,6 - ditertiarybutyl-4-methylphenol 1  
Reaction product of P<sub>2</sub>S<sub>5</sub>-turpentine 0.8  
Mineral lubricating oil Balance

20 2. A non-ash containing lubricating oil composition for aviation engines consisting essentially of a mineral lubricating oil having incorporated therein from about 0.5 to 1% of a reaction product of P<sub>2</sub>S<sub>5</sub>-turpentine and from about 0.5 to 3% of 2,2'-methylene bis(4-methyl-6-tertiarybutylphenol).

25 3. A non-ash containing lubricating oil composition for aviation engines consisting essentially of a mineral lubricating oil having incorporated therein from about 0.5 to 1% of a reaction product of P<sub>2</sub>S<sub>5</sub>-pinene and from about 0.5 to 3% of 2,2'-methylene bis(4-methyl-6-tertiarybutylphenol).

30 4. A non-ash containing lubricating oil composition for aviation engines consisting essentially of a mineral lubricating oil having incorporated therein from about 0.5 to 1% of a reaction product of P<sub>2</sub>S<sub>5</sub>-pinene and from about 0.5 to 3% of 2,6-ditertiarybutyl-4-methylphenol.

35 5. A non-ash containing lubricating oil composition for aviation engines consisting essentially of a mineral lubricating oil having incorporated therein from about 0.5 to 1% of a reaction product of P<sub>2</sub>S<sub>5</sub>-pinene and from about 0.5 to 3% of 2,6-ditertiarybutyl-4-methylphenol.

40 6. A non-ash containing lubricating oil composition for aviation engines consisting essentially of a mineral lubricating oil having incorporated therein from about 0.1 to 5% each of a reaction product of P<sub>2</sub>S<sub>5</sub>-pinene and of 2,6-ditertiarybutyl-4-methylphenol.

45 7. A non-ash containing lubricating oil composition for aviation engines consisting essentially of a mineral lubricating oil having incorporated therein from about 0.1 to 5% each of a reaction product of P<sub>2</sub>S<sub>5</sub>-turpentine and of 2,6-ditertiarybutyl-4-methylphenol.

50 8. A non-ash containing lubricating oil composition for aviation engines consisting essentially of a mineral lubricating oil having incorporated therein from about 0.1 to 5% each of a reaction product of P<sub>2</sub>S<sub>5</sub>-pinene and of 2,4,6-tri-alkylphenol, at least one of the alkyl radicals ortho to the hydroxyl group being a tertiary alkyl radical.

55 9. A non-ash containing lubricating oil composition for aviation engines consisting essentially of a mineral lubricating oil having incorporated therein from about 0.1 to 5% each of a reaction product of P<sub>2</sub>S<sub>5</sub>-turpentine and of 2,4,6-tri-alkylphenol, at least one of the alkyl radicals ortho to the hydroxyl group being a tertiary alkyl radical.

60 10. A non-ash containing lubricating oil composition for aviation engines consisting essentially of a mineral lubricating oil having incorporated therein from about 0.1 to 5% each of a

reaction product of  $P_2S_5$ -terpene and of 2,4,6-trialkylphenol, at least one of the alkyl radicals ortho to the hydroxyl group being a tertiary alkyl radical.

11. A non-ash containing lubricating oil composition for aviation engines consisting essentially of a mineral lubricating oil having incorporated therein from about 0.1 to 5% each of a reaction product of  $P_2S_5$ -turpentine and of 2,2'-methylene bis(4-alkyl-6-tertiaryalkylphenol).

12. A non-ash containing lubricating oil composition for aviation engines consisting essentially of a mineral lubricating oil having incorporated therein from about 0.1 to 5% each of a reaction product of  $P_2S_5$ -turpentine and of 2,2'-alkylidene bis(4-alkyl-6-tertiaryalkylphenol).

13. A non-ash containing lubricating oil composition for aviation engines consisting essentially of a mineral lubricating oil having incorporated therein from about 0.1 to 5% each of a 20 reaction product of  $P_2S_5$ -terpene and of 2,2'-alkylidene bis(4-alkyl-6-tertiaryalkylphenol).

14. A non-ash containing lubricating oil com-

position for aviation engines consisting essentially of a mineral lubricating oil having incorporated therein from about 0.1 to 5% each of a phosphorus sulfide-terpene reaction product and of a trisubstituted phenol selected from the group consisting of 2,4,6-trialkylphenol, at least one of the alkyl radicals thereof ortho to the hydroxyl group being a tertiary alkyl radical and 2,2'-alkylidene bis(4-alkyl-6-tertiaryalkylphenol).

15. A non-ash containing lubricating oil composition for aviation engines comprising a mineral lubricating oil having incorporated therein 0.8% of a reaction product of pinene with  $P_2S_5$  and 1% of 2,6-di-tertiary-butyl-4-methyl phenol.

References Cited in the file of this patent

UNITED STATES PATENTS

| Number    | Name     | Date          |
|-----------|----------|---------------|
| 2,257,872 | Trautman | Oct. 7, 1941  |
| 2,486,188 | May      | Oct. 25, 1949 |
| 2,489,249 | Adelson  | Nov. 29, 1949 |
| 2,493,217 | Berger   | Jan. 3, 1950  |